

Dec. 25, 1945.

C. E. SORENSEN

2,391,523

METHOD FOR CASTING ROTORS

Filed March 31, 1941

*Fig. 1.*



*Fig. 3.*

*Fig. 2.*



*Fig. 4.*



*Fig. 5.*



*Fig. 6.*



Charles E. Sorenson  
INVENTOR.

Edwin C. McRae  
Robert T. Harris  
ATTORNEYS.

WITNESS  
William Jilly

BY

## UNITED STATES PATENT OFFICE

2,391,523

## METHOD FOR CASTING ROTORS

Charles E. Sorensen, Detroit, Mich., assignor to  
 Ford Motor Company, Dearborn, Mich., a corporation of Delaware

Application March 31, 1941, Serial No. 386,033

3 Claims. (Cl. 22—200.5)

This invention relates to the manufacture of cast articles and, more specifically, to methods and molds for use in the centrifugal casting of various articles.

It will be understood that by centrifugal casting is meant the process in which molds are rotated for the purpose of distributing molten metal therein by centrifugal force. This results in an improved metallurgical structure; and, in addition, permits the casting of objects which could not be made by prior methods of casting.

In connection with such centrifugal casting, the use of so-called permanent molds has been quite common. These molds are constructed of metal or other substances which are more or less permanent as compared with the conventional green sand or core molds used in the general casting process and which may be used but once. While these molds may be used a number of times before being damaged by the hot metal, their useful life is limited and considerable effort has been directed to obtaining suitable metals and developing such designs as would permit a longer use of such molds. It is obvious that the more times the mold may be used, the greater will be the economy in the process. It is a further consideration that such molds may be repaired, or damaged parts replaced, easily and cheaply. Apart from this, it is necessary that such a mold be easily assembled or set up preliminary to pouring, and that it be easily disengaged from the cast article after the poured metal has solidified.

The foregoing, as applying both to the centrifugal casting process and the use of permanent molds, represents matters which have been the subject of considerable attention in the prior art. Thus, the general method of centrifugal casting is to set up a mold on a rotatable table, rotate the table at a suitable speed, and then to pour molten metal into the rotating mold. The centrifugal force imparted to the molten metal by the rotating mold is sufficient to force the metal throughout the said mold and will insure a particularly dense structure in the outer parts of such casting. This process has been found adapted to such articles as car wheels, gear blanks and the like in which a high peripheral density is desired. Indeed, when centrifugal casting is used it is found that articles which were formerly thought to be necessarily forged or machined can be made by casting. In such instances, the process results in a substantial economy in both time and material.

This general method does have limitations and has been found unsuitable for articles such as are

described hereinafter, but for which the method of this invention is practicable.

As an illustration of the type of work to which this process may be applied, the impeller of a supercharger is shown. This particular impeller is designed for use in an aircraft supercharger in which it operates at extremely high rotational speed. Up to now, it was thought necessary to form these impellers by forging or machining. 5 This is a lengthy process; and, moreover, these methods necessarily limit the curvatures and the clearances which may be used. On the contrary, in using centrifugal castings, I find that this impeller can be made from a high-strength aluminum alloy, that there is no limitation upon the shape of the blades as no machining is necessary, and that they may be turned out easily and quickly. It will be noted that the vanes of the impeller are of very thin section and it is here that 10 this method of centrifugal casting has a particular advantage.

Considerable effort has also been expended in improving permanent molds from the standpoint of the metal used, the design, suitable facing 15 agents to prevent the adherence of the metal to them and the easy stripping from the cast article. However, it is obvious that in any mold which is alternately subjected to high and low temperatures and which will, as a consequence, expand 20 and contract with each use, failure must necessarily occur eventually. In addition, such molds were generally designed so as to have one surface 25 in contact with the metal and others in contact with the atmosphere. This also set up stresses 30 in the molds during the pouring operation and contributed to their failure. In still other designs, the problem of the expansion of the mold 35 presented serious difficulties. The mold of this invention, which is also shown as applying to 40 the impeller, avoids these difficulties and defects.

An advantage of the process of this invention is that by following it, articles may be cast satisfactorily which heretofore have been considered 45 unsuited for such procedure. It is a further advantage that such articles may be produced more quickly and more cheaply than heretofore. It is a further object of this casting process to extend the benefits of centrifugal casting to articles of 50 relatively small section and to the use of the lighter alloys therein.

An object of the mold of this invention is to provide a mold of the permanent type which may be readily assembled and disassembled. A further object is to construct a mold of interchangeable 55 parts by which failure of any one of the parts

may be immediately replaced without scrapping the mold as a whole. Another object is to design a mold in which proper compensation may be made for temperature changes and the expansion or contraction incident thereto. A further object is to design a mold in which, insofar as possible, temperature stresses in the individual elements of the mold may be equalized.

With these and other objects in view, my invention consists in the arrangement, construction and combination of the various parts of my improved device, as described in this specification, claimed in my claims, and illustrated in the accompanying drawing, in which:

Figure 1 is a perspective view of one of the chills used in assembling the mold of this invention.

Figure 2 is a plan view on a reduced scale of the mold carrier showing a chill in place.

Figure 3 is a plan view of the impeller as cast in the mold of this invention.

Figure 4 is an elevation of the impeller.

Figure 5 is a transverse section taken on the line 5—5 of Figure 2.

Figure 6 is a transverse section taken through the spinner unit used in making the centrifugal casting.

Referring now to the drawing, Figure 3 represents a plan view of an impeller 7 for a super-charger, having a plurality of blades 8 and a hub 9. In the present case, it is cast from an aluminum alloy having a melting point of about 1200° at a pouring temperature of about 1500°. This impeller when so made, using this alloy, the mold of this invention, and the method outlined herein, will be suited for service in cases where heretofore only forged or machined construction has been satisfactory. Moreover, by casting it, such vane shapes as are desired may be obtained without limitation thereon due to the necessity of machining. Finally, these impellers may be produced cheaply and quickly and with a great degree of uniformity.

To accomplish this, the centrifugal casting apparatus shown in Figures 2, 5 and 6 is used in which 10 indicates a mold ring and 11 a mold spinner. The former includes a dish-shaped recess 12 and a peripheral flange 13. The mold spinner includes the complementary flange 14, designed to seat within the peripheral flange 13 of the mold ring, and is provided with a centrally-disposed recess 15. The bottom of the mold spinner is formed with a collar 16 which fits over and is releasably secured to the spinning shaft 17 as by the pin 18.

The chills from which the mold is built up are indicated generally at 19 in Figure 1. Inspection of Figures 3 and 4 will indicate generally the required molding conformation of these chills, since the molding portion of each chill occupies the space between two adjacent impeller blades, as indicated by the centerline 28 in Figure 4.

It will be understood, of course, that the design of the impeller dictates the conformation of the chill to be used; and that a chill to form any desired impeller design may be made, the only limitation being that it may be removable from the impeller after casting.

Referring to Figure 1, it will be seen that the chill 19 has parallel upper and lower surfaces 20 and 21, respectively, and each of these surfaces represents a part of a circular sector. The inner surface 22 of the chill conforms to the exterior of the impeller hub between the vanes. The outer surface 23 of the chill is designed to bear against the wall of the recess 12 in the mold ring. One

side of the chill 24 is formed with a recess 25; the depth of this recess conforms to the thickness of the impeller blade and its outer line 26 follows the configuration of the edge of the impeller blade. The other side 27 does not have such a recess.

As the impeller under consideration has eighteen vanes, eighteen of these chills will be required. These chills are assembled in the mold ring as indicated in Figure 2. One of these chills is there shown in position, with its lower surface 21 resting on the base of the recess 12 and its outer surface 23 bearing against the wall of the recess. Another chill is then placed and its far side 27 bears against unrecessed portion of side 24 of the first chill. Other chills are then added one after the other until all eighteen are placed, the recessed side 24 of the last chill placed contacting the far side 27 of the first chill placed. The centerline 28 on Figure 4 indicates the relationship of one such chill to the impeller as poured.

It is obvious that the chills now cooperate to form a mold for an impeller such as is shown. The outline formed by these assembled chills is indicated in Figure 5, although the configuration of individual chills is not shown.

The spinner 11 is then removed from the shaft 17, is inverted and placed over the mold ring 10, and clamps are applied around the edges of the spinner and the ring to hold them together. This assembly is then inverted, the spinner is re-engaged with the shaft, and the mold is now ready to be poured.

It will be noted that an internally-flared pouring opening 29 is provided which is so shaped to prevent the molten metal from being thrown out of the mold ring during the casting process. The assembled mold is now preheated, it having been found that temperatures from 200° to 800° thereof are preferred before the actual pouring is begun. Molten metal is now introduced through the pouring opening 29 in quantities sufficient to fill the recess 15 and a substantial portion of the recess 30 formed by the assembled chills. As soon as this metal is poured, the rotating mechanism is started and the mold is rotated at a rate of from 700 to 1200 R. P. M. This rotation, of course, impels the molten metal by centrifugal force to flow into and fill the interstices between the chills, thus forming the impeller blades. As a light alloy is used, the rotational speed is somewhat higher than used for iron. Those skilled in this art will recognize that by introducing the molten metal when the mold is at rest and thereafter rotating the mold, a departure is made from the usual practice. Insofar as can be determined, heretofore the molten metal has been added when the mold was revolving and at once projected outward by centrifugal force. In using the earlier method for casting thin sections, the metal fills up these thin parts irregularly; and, as a result, the same effect is achieved as though metal were forced into the thin sections in distinct slugs. These slugs harden in place individually and do not bond together. As a result, blades so cast have been found to consist of successive strips of metal and are not homogenous.

By first providing a pool of molten metal and then commencing the rotation of the mold, it is believed that the metal as a mass is impelled toward the circumference of the mold rather than disconnected slugs being forced therein. When the metal is forced in such a mass, a homogenous blade results and there is no evidence of the

lack of bond displayed in castings made as first described. Following this method, one can cast articles having extremely thin section and obtain a sound and durable product with all of the advantages naturally inherent in centrifugal castings.

Referring now to the mold, it will be seen that this is formed by the cooperating chill parts or sectors. Furthermore, due to the recesses 25 in the individual chills, the molten metal does not reach the upstanding wall of the mold ring. By this means, the serious problems usually met with in the expansion of the circumferential ring are avoided as any expansion circumferentially can be taken up between the individual chills which fit within the ring with a small clearance. Further, it will be noted that each chill has molten metal on each of its sides. This means that there will be no tendency toward cracking or disintegration within the chill itself such as is found in most molds in which one side is exposed to the molten metal and the other side to a much cooler medium. Finally, these chills are interchangeable, and in the event of the failure of one of them, it is only necessary to replace it with a spare chill such as may be kept on hand. It is thus evident that the mold is very cheap to maintain and that it may be kept in such a state as to form perfect castings without extensive repair or machining.

After the mold has been poured, as indicated above, the clamps securing the mold ring to the spinner may be removed and the mold ring lifted therefrom and inverted. The mass therein, which comprises the cast metal and the chills, may then be freed from the mold ring. Suitable pull-out holes 31 are located on the outer surface 23 of each chill and are threaded to receive a pull-out tool. Ordinarily, the chill may be loosened sufficiently to draw it from the casting by tapping it slightly; but if this fails, the pull-out tool can be threaded into the mold and more pressure applied. When the chills are withdrawn, the resulting casting may be machined to its final external dimensions. The chills may then be replaced in the mold ring as indicated above and the procedure repeated. It is obvious that this is particularly adapted to quantity production since successive castings will not only have a high finish, due to the use of the permanent molds, but will also agree within close tolerances. The matter of finish is important, inasmuch as these impellers are designed to rotate at very high speeds, and due to their shape the vane surfaces cannot be readily machined. However, these surfaces may be smoothed by injecting a suitable abrasive in air being pumped by the impeller or by using a regular buffering wheel and it will be found that a very high finish results.

I have thus evolved a method of casting which is of particular use with the mold described; and both method and mold are of particular advan-

tage in forming articles with thin and complex sections such as are illustrated. The advantages of each of these and of both in combination should be apparent at once as described herein.

5 Some changes may be made in the arrangement, construction and combination of the various parts of my improved device without departing from the spirit of my invention and it is my intention to cover by my claims such changes as may reasonably be included within the scope thereof.

I claim as my invention:

1. The method of forming impellers, fans, and the like which comprises, the steps of arranging sector mold parts upon a horizontal rotatable support having a centrally disposed reservoir, a portion of each of said mold sector conforming to the interstices between the vanes of said impeller, the remainder of each said mold sector cooperating with adjacent mold sectors to form a peripheral wall, preheating the mold, pouring an excess of molten metal into said reservoir in the central part of the mold, and then rotating the mold at a speed sufficient to impel the metal substantially instantly and continuously to the remote parts of the mold.

20 2. The method of forming impellers, fans, and the like which comprises, the step of arranging interchangeable mold sectors upon a horizontal rotatable support having a reservoir therein, the inner portion of each said mold sector conforming to the interstices between the vanes of the said impeller, the outer portion of each said mold sector cooperating with adjacent mold sectors to form a peripheral wall, inner faces of said mold sectors conforming to the hub surface of said impeller, preheating the mold, pouring an excess of molten metal into the central portion of the mold and the reservoir, and then rotating the mold at a speed sufficient to impel the metal substantially instantly and continuously to the remote parts of the mold.

25 3. A method of centrifugally casting articles having a central portion and a plurality of elements of reduced section extending outwardly therefrom, which comprises, the steps of arranging a mold having a central mold cavity defining said central portion and extending mold cavities connected to said central mold cavity defining said elements and having a central reservoir in communication with said central mold cavity and positioned beneath the connection between said central and extending mold cavities, pouring an excess of molten metal in said mold to form a pool therein, said pool filling said reservoir and a portion of said central mold cavity, and thereafter rotating said mold to force said molten metal substantially instantaneously into the remote parts of said mold, said reservoir remaining filled with metal throughout the casting operation.

CHAS. E. SORENSEN.